



US005490969A

# United States Patent [19]

Bewlay et al.

[11] Patent Number: 5,490,969

[45] Date of Patent: Feb. 13, 1996

[54] MOULD FOR ISOSTATIC PRESSING

[75] Inventors: **Bernard P. Bewlay; Dennis J. Dalpe**,  
both of Schenectady, N.Y.[73] Assignee: **General Electric Company**,  
Schenectady, N.Y.

[21] Appl. No.: 269,272

[22] Filed: Jun. 30, 1994

[51] Int. Cl.<sup>6</sup> B22F 3/02; B22F 5/00

[52] U.S. Cl. 419/68; 419/66

[58] Field of Search 419/66, 68

## [56] References Cited

## U.S. PATENT DOCUMENTS

|           |         |                 |       |           |
|-----------|---------|-----------------|-------|-----------|
| 1,510,745 | 10/1924 | Montgomery      | ..... | 419/66    |
| 3,311,685 | 3/1967  | Forney et al.   | ..... | 264/111   |
| 3,571,854 | 3/1971  | Lundstrom       | ..... | 18/16.5   |
| 3,577,635 | 5/1971  | Bergman et al.  | ..... | 29/615    |
| 3,850,567 | 11/1974 | Heier           | ..... | 425/405 R |
| 4,271,114 | 6/1981  | Ohno            | ..... | 264/114   |
| 4,834,940 | 5/1989  | Krall           | ..... | 419/66    |
| 4,943,319 | 6/1990  | Yanagawa et al. | ..... | 75/229    |
| 5,019,330 | 5/1991  | Bewlay et al.   | ..... | 419/39    |
| 5,057,273 | 10/1991 | Hanson          | ..... | 419/68    |
| 5,085,828 | 2/1992  | Shain et al.    | ..... | 419/66    |

## OTHER PUBLICATIONS

"Tooling for Cold Isostatic Pressing," KJ Morris, Isostatic Pressing Technology, edited by PJ James, Applied Science Publishers, New York, Chapter 4, pp. 91-119.

Primary Examiner—Donald P. Walsh

Assistant Examiner—Scott T. Bluni

Attorney, Agent, or Firm—R. Thomas Payne; James Magee, Jr.

## [57] ABSTRACT

Methods for forming compacts having reduced elephant's foot effect are disclosed. The apparatus utilized includes a press for dry bag isostatic pressing, the press body having a cavity with at least one open end formed therein, an elastic mould, operatively positioned inside the cavity for compacting metal powder, means, operatively connected to the mould for expanding the mould and compacting the metal powder, and at least one press member having a base section substantially normal to the cavity and an insert section extending from base section into the cavity, the insert section being formed in the shape of any one of a plurality of geometric shapes. The method comprises depositing a metal powder in the cavity of a cold isostatic press, sealing at least one end of the cavity with a punch having a section substantially normal to the cavity and an insert section having any one of a plurality of geometric shapes extending from the base section into the cavity, applying pressure to the outer surface of the mould, decompressing the mould by reducing the pressure applied in a controlled manner and removing the resulting compact from the mould, the compact having a taper applied to at least one end which reduces the elephant's foot effect.

14 Claims, 3 Drawing Sheets





fig. 1  
(PRIOR ART)



**fig. 2a**

(PRIOR ART)



**fig. 2b**

(PRIOR ART)



**fig. 3**



## MOULD FOR ISOSTATIC PRESSING

## BACKGROUND OF THE INVENTION

This invention generally relates to methods for dry bag cold isostatic pressing, and more particularly to methods utilizing dry bag cold isostatic press moulds having improved punches for sealing the mould ends of such so as to produce a compact having a reduced elephant foot effect at the ends of the compact.

Metal powder, such as tungsten, is typically disposed in a cylindrical elastic mould and radially compacted. An apparatus for performing such radial compaction operations is well known in the art as a dry bag cold isostatic press. See "Isostatic Pressing Technology", edited by P. J. James, Applied Science Publishers, New York, Chapter 4, "Tooling for Cold Isostatic Pressing", pp. 91-119, incorporated herein by reference, dry bag cold isostatic pressing is sometimes herein referred to as dry bag pressing.

In dry bag pressing, an elastic bag or mould is fixed within a pressure vessel. The elastic mould has at least one open end which is sealed with the pressure vessel so that the fluid pressure medium within the vessel cannot enter the mould interior. The elastic mould is made from a material which does not chemically react with either the powder or the pressure medium, and readily releases from the powder compact. A material having a high resistance to wear from the powder is also desirable. Mould materials that can be used include natural rubber, neoprene, polyvinyl chloride, butyl, nitride, silicone, and preferably urethane.

In one method of dry bag pressing, a cylindrical elastic mould is used that is open at both ends, and has a void space, such as, for example, a cylindrical void therein. Sealing means for the open mould ends are provided by wear resistant metal punches. The punches are located and restrained by the yoke of the press, and guided into the bag by wear resistant bushes mounted in the pressure vessel. The top punch is removed and powder is charged into the void space in the mould completely filling the void space between the sealing means. The powder is charged into the mould by means well known in the art for providing a fill density that does not allow settling of the powder prior to compaction. A powder fill density of at least about 5 grams per cubic centimeter, and preferably about 6 grams per cubic centimeter is adequate. One method for providing such a fill density comprises pouring a small amount of powder in the mould followed by tamping of the powder, and repeating this procedure until the void space is filled.

The top punch is engaged in the mould and a fluid pressure medium is applied to the outside of the mould. The mould is supported by a metal cage or lantern ring which keeps the mould radially located, and distributes the fluid pressure medium evenly around the bag. A pressure of at least about 560 kg/cm<sup>2</sup>, preferably at least about 1760 kg/cm<sup>2</sup>, can be used to compact the powder, for example tungsten. Preferably, the radial pressure is applied for at least about 30 seconds to densify the powder to at least about 50 percent, preferably at least about 60 percent of theoretical density. Such compaction provides significant strength to the compact so that it can be easily handled and has sufficient structural strength to withstand the resistance sintering operation, without breakage.

The radial pressure applied to the mould by the fluid pressure medium is slowly removed in a controlled fashion to provide a controlled decompression of the compact. An

uneven decompression of the compact may result in cracking or breakage of the compact. Pressure can be reduced at a rate up to about 70 kg/cm<sup>2</sup>/second, preferably up to about 11 kg/cm<sup>2</sup>/second to prevent such cracking or breakage of the compact.

The internal diameter of the void space in the mould is dependent upon the compaction ratio of the powder to be pressed. The compaction ratio and internal diameter are determined by means well known in the art to form a compact of the desired diameter. Such methods are described, for example, in "Tooling for Cold Isostatic Pressing" referenced above. For example, a tungsten compact of about 22 millimeters in diameter can be formed from a mould having an internal void space of 30.5 millimeters in diameter.

A tendency toward flaring of the ends of the formed compact has previously been minimized by careful adjustment of the inner surface profile in the mould. The punches sealing the ends of the cylindrical mould were provided to have a smaller diameter than the internal void space diameter of the cylindrical mould. The ends of the mould which seal around the punches are formed to correspond to the smaller diameter of the punches. The internal void space then has a small tapered section adjacent the punches tapering from the smaller diameter of the punches to the larger diameter of the void space.

The pressed compact is removed from the mould and sintered by resistance heating. As an example for tungsten, a resistance heating current of about 4,000 to 6,500 amps is transmitted through the compact according to cycles well known in the art. For example see "Application of Tungsten Wire as the Light Source in Incandescent Electric Lamps," D. J. Jones, Metallurgy and Material Technology, Volume 5 No. 10, pp. 503-512, 1973. Such resistance heating is sufficient to heat the compact to between about 2,100° and about 3,000° C. where the compact is sintered to about 85 percent of theoretical density. Other metals and ceramics compacts can be sintered by well known conventional methods.

However, solid rods of tungsten or other powder which are compacted by cold isostatic pressing typically have a cylindrical flared or "elephant's foot" region at each end due to friction between the punch and the powder. These elephant's feet have been found to generate significant yield reduction after either pressing or sintering; thus, indicating that "elephant's foot" is a major limitation in the efficient production of metal compacts by cold isostatic pressing.

Notwithstanding, the presentation of the art disclosed above, there continues to be a need for improved methods to eliminate or reduce cylindrical flared or "elephant's foot" regions at each end of powder, such as tungsten, compacted by cold isostatic pressing. Such methods desirably will provide increased product yield of both pressed and sintered articles while eliminating the need for the careful adjustment of the inner surface of the profile in the mould; would have a punch profiled in a geometric shape that would either eliminate or at least significantly reduce the elephant's foot region at least one end; would, in particular, reduce the diameter of at least one end region of the pressed compact during cold isostatic pressing; and would eliminate or at least significantly reduce the elephant's foot by having a taper applied at one or both ends of the cold isostatic pressed compact.

## SUMMARY OF THE INVENTION

In carrying out the present invention in preferred forms thereof, we provide methods for the cold isostatic press

production of metal compacts, such as tungsten.

The present invention can be used to change the end geometry of articles produced by cold isostatic pressing from an axi-symmetric to a tapered form. This is accomplished by modification of the punches at one or both ends of the mould to any one of a plurality of geometric shapes such as, for example, a semi-circular notch or a tapered notch.

Each method of the present invention includes the utilization of an isostatic press for producing a cylindrical or otherwise shaped compact. The apparatus utilized includes a press which comprises a pressure vessel, a top and a bottom punch, an elastic mould bag, (a lantern ring), which keeps the mould bag radially located and distributes the fluid pressure evenly around the bag, an isostatic fluid port formed in the pressure vessel as well as a fluid bleed means. At each end of the apparatus are top and bottom members upon which the top and bottom punches are respectively operatively connected. The punches are modified to provide a surface contacting the pressed compact other than two surfaces perpendicular to the center line of the mould cavity so that elephant foot is eliminated on at least one side of one end of the resulting compact.

One method, according to the present invention includes a method for forming a metal compact in a cold isostatic press having at least one open end, comprising the steps of: depositing a metal powder in the cavity of the cold isostatic press; sealing at least one end of the cavity with a punch having a section substantially normal to the cavity and an insert section, having a plurality of geometric shapes, extending from the base section into the cavity; applying pressure to the outer surface of the mould; and decompressing the mould by reducing the pressure over time such that the resulting compact has a taper applied to at least one end thereof.

Another method according to the present invention includes a method for forming a metal compact in a cold isostatic press having two open ends, comprising the steps of: depositing a metal powder in the cavity of the cold isostatic press; sealing both ends of the cavity with a punch having a section substantially normal to the cavity and an insert section, each having any one of a plurality of geometric shapes, extending from the base section into the cavity; applying pressure to the outer surface of the mould; and decompressing the mould by reducing the pressure over time such that the resulting compact has a taper applied to each end thereof.

In one specific method of the present invention, at least one punch has been formed as a semi-circular notch.

In another specific method, at least one punch has been formed as a tapered notch.

In still another aspect of the present invention a metal compact is prepared in a cold isostatic press having two open ends and a cavity by a process comprising the steps of: depositing a metal powder in the cavity of the cold isostatic press; sealing both ends of the cavity with a punch having a section substantially normal to the cavity and an insert section, each having any one of a plurality of geometric shapes, extending from the base section into the cavity; applying pressure to the outer surface of the mould; and decompressing the mould by reducing the pressure in a controlled manner such that the resulting compact has a taper applied to each end thereof.

Accordingly, an object of the present invention is to provide a method for modification of at least one end of both solid rod and tubular articles produced by cold isostatic

pressing utilizing any one of a range of end geometry's on one or both ends of the produced article.

Another object of the present invention is to provide a method for producing compacts by cold isostatic pressing having greater yields than those previously produced.

Still another object of the present invention is to provide a method that reduces the end diameter of the end region of a compact manufactured by dry bag and wet bag cold isostatic pressing.

Other objects and advantages of the invention will be apparent from the following description, the accompanying drawings and the appended claims.

#### BRIEF DESCRIPTION OF THE DRAWINGS

FIG. 1 is a partial sectional view of an illustrative dry bag tooling press;

FIG. 2a is a sectional view of the press of FIG. 1 showing the press closed and the bag deformed to produce a compact or ingot;

FIG. 2b is a partial sectional view of FIG. 2 showing a prior art method of eliminating the elephant's foot effect;

FIG. 3 is a partial sectional view of the top press member of the present invention having a modified punch member;

FIG. 4 is a partial sectional view showing the illustrated modified punch of FIG. 3 positioned inside an deformed press cavity;

FIG. 5a is a sectional view of a semi-circular punch as used with the methods of the present invention;

FIG. 5b is a sectional view of a tapered punch as utilized with the methods of the present invention;

FIG. 6a is a sectional view of a compact formed by the punch of FIG. 5a; and

FIG. 6b is a sectional view of a compact formed by the punch of FIG. 5b.

#### DETAILED DESCRIPTION OF THE INVENTION

Production of metal compacts or ingots, such as tungsten with tapered ends by ram pressing of metal powder in steel dies is well established. The present invention is directed to a method for making a compact or ingot having improved product yield of both pressed and sintered articles. The present invention includes methods for modifying the end geometry of a compact and in particular, reducing the diameter of the end region of a pressed compact during dry bag and wet bag cold isostatic pressing. A taper can be applied to one or both ends of the compact. The principal advantage of the present invention is that it increases product yield.

The methods of the present invention utilize an improved dry bag tooling press, generally designated 20, is illustrated in FIG. 1. The press 20 comprises a top press member 22, a bottom press member 24, a top punch 26 and a bottom punch 28, which are operatively connected to the respective top 22 and bottom 24 press members. The press body 30 has a cavity 32 formed therein which may be in any desired geometrical shape. The interior walls of the body 30 consists of a mould bag 34. Between the press body 30 and the mould bag 34 is a lantern ring 36. Formed in the press body 30 is an isostatic fluid port 38 and a bleed screw 40. At each end of the cavity are bushings 42 and 44, respectively. The press 20 operates in a conventionally known manner.

Also shown in FIG. 1 inside the cavity 32 is the uncom-  
pressed metal powder 46 and the compressed compact 50  
(shown in dotted lines) after the application of pressure and  
the completion of the isostatic pressing cycle. The  
“elephant’s foot” or flaring at each end 52 is clearly illus-  
trated in FIG. 1.

FIG. 2a shows the mould bag in its deformed condition  
applying pressure on the metal particles to form the com-  
pact. The prior art method of eliminating the “elephant’s  
foot” or flaring by careful reconfiguring of the internal  
mould bag so that a compact ingot is produced without the  
“elephant’s foot” is illustrated in FIG. 2b.

FIG. 3 illustrates a modified top punch 26 positioned in  
the upper portion of the press 20 of FIG. 1. As clearly  
illustrated, top punch 26 includes an extension 62 which, as  
illustrated in FIG. 4, eliminates the elephant’s foot on that  
particular side thereof. By imparting a notch 63 in the  
compact 50, the elephant’s foot has been eliminated on the  
one side, as illustrated in FIG. 6a.

FIGS. 5a and 5b, illustrate representative punches 70 and  
72. The semi-circular punch 70 has an extension 62 which  
can extend for at least about one-fifth of the length of the  
overall punch which enters into the cavity 32.

FIG. 5b illustrates a tapered punch 72 having an extended  
portion 74 with a depth of approximately half of the overall  
length of the die portion which extends into the cavity 32. As  
illustrated, the angle of wall 76 is about 26 degrees but an  
acceptable angle could be from about 5 to about 82 degrees  
and the length of end 78 is about 0.174 the width of the  
punch 72 but an acceptable length could be from about 0.001  
to about 0.25 the width of the punch 72. By imparting the  
taper 78 in the compact 50, as illustrated in FIG. 6b, once  
again the elephant’s foot has been eliminated on the one  
side.

The methods of the present invention will be better  
understood by referring to the following examples illustrat-  
ing the methods thereof.

#### EXAMPLE I

In one application of the methods of the present invention,  
a charge of 1450 g of tungsten powder with a mean particle  
size of 4.5  $\mu\text{m}$  was poured into a flexible tubular urethane  
mould which had been sealed previously at the bottom with  
a steel punch of the design shown in FIG. 5a. The urethane  
mould had previously been fixed in a dry bag cold isostatic  
press. The mould had an internal diameter of 23 mm and an  
internal length of 660 mm. The top of the mould was sealed  
with a punch of a similar design after powder filling. The  
mould can be filled with powder either manually or auto-  
matically or is known in the art.

A pressure of 170 MPa was applied to the mould using  
hydraulic fluid, held for 60 seconds, and then released. After  
decompression, the pressed tungsten compact or ingot was  
removed from the mould. The mean diameter of the pressed  
rod was 15.6 mm, neglecting the bottom and top 50 mm of  
the ingot. Each end was tapered in a manner controlled by  
the profile of each punch, as illustrated in FIG. 5a.

The ingot can then be sintered directly by self-resistance  
heating, or indirectly in a furnace. The punch material which  
is used to modify the ingot end can be either steel or  
urethane. Urethane has the advantage of preserving the  
isostatic mode of compaction in the end regions of the ingot  
but has the disadvantage of making decompression slower  
and control more difficult.

In another mode of operation, a similar procedure to that  
of Example I was used together with tungsten powder with  
a mean particle size of 1.9  $\mu\text{m}$ . The mean diameter of the  
ingot pressed at 170 MPa was 13.5 mm and each end was  
tapered in a similar manner to the ingot shown in FIG. 6b  
utilizing the punch of FIG. 5b. It is believed that ingots with  
end tapers can be pressed in this manner from such powder  
using pressures between about 20 and about 211 MPa.

#### EXAMPLE II

In an additional example of the methods of the present  
invention, ingots were pressed with notched ends using the  
punches illustrated in FIG. 5a. The notched end 62 of the  
ingot occupied between 5 and 60% of the diameter of the  
punch 70. In one mode, a punch which had a notch 62 13  
mm deep and 50% of the cross sectional area of the ingot  
was used. The ingot was pressed from 4.5  $\mu\text{m}$  powder using  
the procedure described earlier with a pressure of about 170  
MPa.

The resulting ingot is illustrated in FIG. 6a. The length of  
the notch 63 can be from 1% to 10% of the length of the  
ingot. The notch can be pressed into one or both ends of the  
ingot. The semi-circular notches can be pressed so that they  
are parallel with, perpendicular to and in any orientation  
with respect to each other. Generally, the notches are dis-  
posed 180° with respect to each other on the opposite ends.

Ingot end modification helps to reduce end losses during  
further processing. For example, ingot end tapering is partic-  
ularly valuable for self resistance sintering where water  
cooled electrodes are attached to the ingot ends. The cooling  
effect of the electrodes reduces sintering at the ingot ends.  
Reduction in the cross sectional area can be used to increase  
the local current density and therefore the rate of heat input  
to the end of the ingot and thereby overcome the cooling  
effect of the electrodes. In this manner, more uniform  
sintering is generated along the full length of the ingot. The  
methods of the present invention provided a flat surface  
pressed onto the end of the ingot. This flat surface aids the  
application of electrodes to the ingot for self resistance  
sintering.

The methods of the present invention can be used for a  
range of powders including both metallic powders, such as,  
for example, tungsten, tantalum, molybdenum, and copper,  
as well as ceramic powders such as for example, alumina,  
zirconia and yttria.

While the methods herein described constitute preferred  
methods of the invention, it is to be understood that the  
invention is not limited to these precise methods and  
changes may be made therein without departing from the  
scope of the invention which is defined in the appended  
claims.

What is claimed is:

1. A method for forming a metal compact in a cold  
isostatic press having at least one open end comprising the  
steps of:

depositing a metal powder in the mould of the cold  
isostatic press;

sealing at least one end of the mould with a punch having  
a base section substantially normal to the mould and an  
insert section, having any one of a plurality of geomet-  
ric shapes, extending from the base section into the  
mould;

applying pressure to the outer surface of the mould; and  
decompressing the mould by reducing the pressure such  
that the resulting compact has a taper applied to at least

- one end thereof thereby eliminating elephant's foot on the tapered end.
2. The method of claim 1 further comprising the step of: removing the resulting compact from the press.
3. The method of claim 1 wherein the press has a mould having two open ends and the sealing step is accomplished by two punches having any one of a plurality of geometric shapes.
4. The method of claim 1 wherein the insert section extending from the base section has a semi-circular shape.
5. The method of claim 1, wherein the insert section extending from the base section has a tapered shape.
6. A method for forming a metal compact in a cold isostatic press having two open ends, comprising the steps of:
- depositing a metal powder in the mould of the cold isostatic press;
- sealing each end of the mould with a punch having a base section substantially normal to the mould and an insert section, each insert section having any one of a plurality of geometric shapes, extending from the base section into the mould;
- applying pressure to the outer surface of the mould; and decompressing the mould by reducing the pressure such that the resulting compact has a taper applied to each end thereof thereby eliminating elephant's foot on each end.
7. The method of claim 6 further comprising the step of: removing the resulting compact from the press.
8. The method of claim 6 wherein at least one punch extension has a semi-circular shape.

9. The method of claim 6, wherein at least one punch extension has a tapered shape.
10. A metal compact prepared in a cold isostatic press having at least one open end by a process comprising the steps of:
- depositing a metal powder in a mould of the cold isostatic press;
- sealing at least one end of the mould with a punch having a base section substantially normal to the mould and an insert section, having a plurality of geometric shapes, extending from the base section into the mould;
- applying pressure to the outer surface of the mould; and decompressing the mould by reducing the pressure such that the resulting compact has a taper applied to at least one end thereof.
11. The compact of claim 10 wherein the process further comprises the step of:
- removing the resulting compact from the press.
12. The compact which results from the process of claim 10 wherein the press has a mould having two open ends and the sealing step is accomplished by two punches having any one of a plurality of geometric shapes.
13. The compact which results from the process of claim 10 has a taper from a semi-circular punch extension which forms the taper.
14. The compact which results from the process of claim 10 has a taper from a tapered shaped punch extension.

\* \* \* \* \*